

1

3,399,177

**CRIMPABLE FIBRES OF ACRYLONITRILE/N-METHYLOL ACRYLAMIDE COPOLYMERS**

Frank Reeder and James Dennis Griffiths, Coventry, England, assignors to Courtaulds Limited, London, England, a British company

No Drawing. Filed June 9, 1964, Ser. No. 373,876  
Claims priority, application Great Britain, June 13, 1963,  
23,572/63

4 Claims. (Cl. 260—85.5)

This invention is concerned with inherently crimped or crimpable fibres in the form of staple fibres, continuous filaments, spun yarns or continuous filament threads and extends to knitted and woven goods incorporating such fibres.

It has been proposed to make crimpable polyacrylonitrile fibres by imposing an asymmetric cross-section on the fibres. According to one proposal, a fibre is composed of two chemically different polymers which occupy discrete collateral zones. The fibres are made by spinning the polymers side by side through each hole of a spinning jet. The polymers respond differently to heat, one shrinking more than the other, so that when the fibre is heated, it is drawn into a helical coil in which the more shrunken polymer follows the shorter path on the inside of the coil.

In a second process, a chemically homogeneous copolymer is extruded through an asymmetric jet hole in which the polymer is subjected to different amounts of shear across the hole. The extruded polymer is immediately coagulated to form a fibre which retains substantially the shape imposed by the jet-hole, and is stretched and dried under tension. The structure of this fibre is asymmetric in the physical properties of the polymer; that part of the polymer which was most highly sheared during extrusion is the most highly orientated and strained part of the fibre and, therefore, the part which shrinks most when the fibre is heated. This fibre, too, assumes a helically coiled configuration when it is heated.

The essence of both processes is the mechanical imposition of a chemical or physical asymmetry on the fibre. It is surprising, therefore, to find a process for making inherently crimped or crimpable fibres which does not rely on imposing asymmetry on the fibres mechanically.

A crimped or crimpable fibre according to the present invention is a fibre of a copolymer containing a major proportion of acrylonitrile and from 7 to 20 mol percent of an N-methylol or a latent N-methylol derivative of an ethylenically unsaturated acid amide.

Wet-spun fibres which are stretched wet and dried under little or no tension, crimp spontaneously during drying, whilst those which are stretched-strained by being dried under tension or stretched after drying, crimp when heated to above their second order transition temperature.

The amide derivative is preferably derived from acrylamide or methacrylamide. N-methylol acrylamide and N-methylol methacrylamide are examples of the derivatives comprising free methylol groups, but we prefer the latent N-methylol derivatives in which the hydrogen of the hydroxyl groups of the N-methylol group is replaced by an alkyl including a hydroxy alkyl group, or a secondary amino group,  $—N(R)_2$ , where R is alkyl, to reduce the chemical activity of the substance at near ambient temperatures, and increase the stability of the polymer during the stages of manufacture and spinning into fibres. The latent N-methylol derivatives must, however, be capable of interacting to cross link the polymer or of generating N-methylol groups which interact to cause cross linking at temperatures above those encountered in earlier process steps i.e. above about 100° C. The preferred, latent N-methylol derivatives are N (methoxy methyl) acrylamide and N (ethoxy methyl) acrylamide and the analogous derivatives of methacrylamide.

2

The fibre may be made using wet- or dry-spinning techniques, although a wet-spinning process is preferable, particularly one in which a solution of the polymer in concentrated sodium thiocyanate solution is extruded into water or dilute sodium thiocyanate solution to form fibres which are stretched by at least 500 percent in hot water or steam. The fibres may then be dried under tension to induce the stretch-strained character, or, after having been dried when relaxed the fibres may be strained by being stretched again. The stretched-strained fibres develop crimp, on being heated, preferably in contact with water or steam, to above their second order transition point which in all cases is less than 100° C.

The spinning process can be made to yield crimped fibres directly if the never-dried fibres are dried under little or no tension.

The polymer solution is homogeneous and may be extruded through circular jet holes so that no asymmetry is imposed mechanically on the fibre.

At the present time there is no completely acceptable theory to account for the ability of the fibres to crimp. It is equally surprising that some fibres have non-circular cross-sections. Fibres made by a wet spinning process from a copolymer having more than 10 percent of N-methylol acrylamide, for example, were found to have a ribbon-like shape in which the width is 5 or 6 times the thickness and the cross-section is flat or curled on itself to a C-shape. It will be understood, however, that the non-circular shape is not an inevitable feature of the fibres of this invention and that some circular cross-sectioned fibres have been made with the ability to crimp.

The fibres of this invention are remarkable also for their ability to shrink when heated. Shrinkages of more than 40 percent and frequently as high as 75 percent have been observed.

The simultaneous shrinking and crimping which the fibres show when heated to above 100° C. has a number of useful applications, amongst which are

- (i) the formation of a bulkier thread of crimped continuous filaments by the application of heat,
- (ii) the formation of a bulkier spun yarn in which the fibres are those of this invention alone or in blend with other and preferably more heat-stable fibres,
- (iii) shrinking and bulking a woven or knitted fabric in the piece or made up into oversized garments.

The crimp can be eliminated from fibres which have been heated only long enough to develop the crimp, merely by stretching. However, it is possible to set the crimp in the fibres by cross-linking and the polymer requires no added reactant in order to do this. The N-methylol amide groups or latent N-methylol amide groups may be condensed intermolecularly to form methylene or dimethylene ether bridges. The condensation is catalysed by acids and some salts, for example those disclosed as catalysts for the reaction of cellulose and formaldehyde in British patent specification No. 930,132. In a preferred polymer, an acidic monomer, for example methallyl sulfonic acid, is incorporated to act as a catalyst for the cross-linking reaction. The cross-linking reaction requires that the fibre incorporating or impregnated with a catalyst is heated and, as heat is also required to develop the crimp, it is possible to combine both steps in a single treatment, particularly as the rate of crimping is so much more rapid than that of condensation reaction, that virtually all the cross-links are formed in the already crimped fibre.

Once the polymer is cross-linked, the crimp proves remarkably stable and is retained or regained during repeated cycles of washing and drying and cycles of tensioning and relaxing.

The invention is illustrated by the following examples in which parts are by weight.

## Example 1

A polymerisation charge was made up of:

|                             | Parts |
|-----------------------------|-------|
| Acrylonitrile               | 315   |
| N-methylol acrylamide       | 107   |
| Azobisisobutyronitrile      | 3.9   |
| Iso-propanol                | 47    |
| Sodium thiocyanate crystals | 1955  |
| Water                       | 572   |

and the pH adjusted to 8. The charge was fed to a tubular reactor and there heated to a temperature of 80° C. The average dwell time of the charge in the reactor was 1½ hours. The charge emerged as a homogeneous, pale, viscous copolymer solution. Analysis showed that 92 percent of the acrylonitrile and N-methylol acrylamide had copolymerised and that the copolymer had an intrinsic viscosity of 1.31.

The copolymer solution was extruded through a 20 hole jet, each hole having a diameter of 0.005 inch into a water bath at ambient temperature to form fibres. The fibres were stretched by 20 times in live steam, collected on a bobbin and dried. The fibres had an average denier of 4.4. The stretching step was modified after the collection of the first sample, to stretching the fibres in water at 87° C. by 12½ times.

The fibres from both stretching operations crimped instantaneously when relaxed in contact with a surface at 120° C.

The fibres were cross-linked by first impregnating them with a 5 percent  $MgCl_2$  solution and finally heating them at 160° C. for 2 hours. When the fibres were relaxed and heated, the crimp was set by the cross-linking to the extent that it could not be removed by straining the fibres. The cross-linked fibres were also, insoluble in a wide variety of liquids, some of which were excellent solvents for the copolymer before cross-linking.

## Example 2

A mixture was formed of:

|                             | Parts |
|-----------------------------|-------|
| Thiourea dioxide            | 2.1   |
| N-methoxy methyl acrylamide | 14.15 |
| Acrylamide                  | 8.85  |
| NaCNS                       | 450   |
| Water                       | 302   |
| Isopropanol                 | 31    |
| Acrylonitrile               | 117   |
| Azobisisobutyronitrile      | 1.4   |

The pH of the solution was adjusted to 6 with a sodium hydroxide solution and more water was added to bring the mixture to a total of 1,000 parts.

Half the mixture was placed in a stirred reactor equipped with a reflux condenser and the temperature of the mixture was raised to 80° C. After 10 minutes, the addition of the remainder of the mixture to the reactor was started and continued at a constant rate over another hour. Heating and stirring were continued for a further 80 minutes, after which unreacted acrylonitrile was removed under vacuum, leaving a clear, pale yellow, viscous solution.

The conversion of monomer to polymer was found to be 92 percent complete and the inherent viscosity of the polymer (in 50 percent w./w. aqueous NaCNS) was 0.90.

The viscous solution was extruded through a 20 hole jet, each hole having a diameter of 0.005 inch, into water at 4° C. to form filaments which were taken up at 2.5 m./m., stretched ten times in steam and collected. The still-wet filaments were subsequently washed with water, impregnated with an 11 percent solution of  $H_3PO_4$  in water and allowed to dry in air in a relaxed condition. The dry filaments were strongly crimped and possessed an asymmetric cross-section. At this stage the filaments could be dissolved in a 50 percent w./w. aqueous NaCNS solution and the crimp could be removed by tensioning

the filaments in live steam. However, after the filaments were cured in a relaxed condition by heating to 150° C. for 4 minutes, the fibre was only slightly swollen by the 50 percent NaCNS solution and the crimp could not be pulled out in steam. The cured fibre had a tenacity of 1.7 grams per denier and an extensibility of 28 percent.

When the freshly-spun fibres were dried under tension they did not develop crimp, but could be made to do so on heating to say 160° C. in a relaxed state at which temperature the filaments may also be cured. Such filaments had a tenacity of 3.12 grams per denier and an extensibility of 13.7 percent.

## Example 3

A polymerisation process and extrusion identical with those described in Example 2, with the exception that the freshly-extruded filaments were stretched by only 5 times in water at 70° C., provided filaments which developed more crimp on air-drying in a relaxed condition.

When the spinning process was altered so that the freshly extruded filaments were stretched by 24 times in steam and the filaments were cured in a relaxed state, the filaments acquired a tenacity of 3.28 grams per denier and an extensibility of 24 percent.

## Example 4

The polymerisation procedure of Example 2 was followed with a mixture having a pH of 6 and composed of:

|                             | Parts |
|-----------------------------|-------|
| Acrylonitrile               | 122   |
| N-methylol acrylamide       | 29.2  |
| Thiourea dioxide            | 2.27  |
| Azobisisobutyronitrile      | 1.51  |
| Isopropanol                 | 31    |
| NaCNS                       | 450   |
| Water to make up a total of | 1000  |

The inherent viscosity of the polymer was 0.87 as determined in 50 percent NaCNS.

The extrusion was similar to that described in Example 2 with the exception that the freshly-extruded filaments were stretched by 26 times, soaked in a 1 percent aqueous solution of  $NH_4Cl$ , before drying in a relaxed condition in air. The dried fibre was highly crimped and could be cured by heating for 4 minutes at 150° C.

## Example 5

The polymerisation process disclosed in Example 2 was used to polymerise the monomers in a charge made up of:

|                             | Parts |
|-----------------------------|-------|
| Acrylonitrile               | 111   |
| N-methylol acrylamide       | 22.5  |
| Acrylamide                  | 8.7   |
| Sodium methalkyl sulphonate | 7.8   |
| Thiourea dioxide            | 2.25  |
| Azobisisobutyronitrile      | 1.5   |
| NaCNS                       | 450   |
| Water to make a total of    | 1000  |

and at a pH of 6.

The resultant viscous solution was extruded through a 40 hole jet, each hole of 0.003 inch diameter, into water at 30° C. The filaments were taken up at 2.5 m./m., stretched 15 times in water at 75° C., washed in dilute sulphuric acid and dried in a relaxed state at 100° C. The filament crimped during the last step, but not to the extent of the filament made by following the procedure of Example 2. At this stage the filament had a tenacity of 1.07 and an extensibility of 43 percent. After curing for 8 minutes at 150° C., the filament had a tenacity of 1.72, an extensibility of 34 percent and an imbibition in 50 percent NaCNS of 23 percent.

## Example 6

The polymerisation process of Example 2 was followed

in preparing a solution of a copolymer of 95 parts of acrylonitrile and 15 parts of N-methylol-acrylamide. The solution was extruded into water at 12° C. to form filaments of circular cross-section which crimped spontaneously when dried relaxed. The filaments formed by extruding the solution into water at 4° C. did not crimp spontaneously.

What we claim is:

1. A chemically and physically homogeneous, inherently crimpable fiber of a copolymer consisting essentially of a major proportion of acrylonitrile and from 7 to 20 mol percent of an N-substituted derivative of acrylamide or methacrylamide, said derivative being chosen from the group consisting of derivatives having N-methylol groups and derivatives capable of forming N-methylol groups on heating to above about 100° C., said copolymer being formed by free-radical copolymerization.

2. A fibre as claimed in claim 1 in a stretch-strained condition.

3. A fibre as claimed in claim 1 in which the latent N-methylol derivative is chosen from the group consisting of N(methoxymethyl) acrylamide, N(ethoxymethyl) methacrylamide and N(butoxy methyl) acrylamide.

4. A fibre as claimed in claim 1, incorporating at least 10 percent of the N-substituted amide and having a ribbon-like shape.

References Cited

UNITED STATES PATENTS

|           |         |                 |          |
|-----------|---------|-----------------|----------|
| 2,560,680 | 7/1951  | Allewelt        | 260—85.5 |
| 2,649,438 | 8/1953  | Bruson          | 260—85.5 |
| 2,796,656 | 6/1957  | Schappel et al. | 161—173  |
| 2,931,091 | 4/1960  | Breen           | 161—173  |
| 3,016,283 | 1/1962  | Schappel        | 264—168  |
| 3,065,042 | 11/1962 | Bradley         | 264—168  |
| 2,718,515 | 9/1955  | Thomas          | 260—85.5 |
| 2,761,856 | 9/1956  | Suen et al.     | 260—85.5 |
| 2,984,588 | 5/1961  | Graulick et al. | 260—85.5 |

FOREIGN PATENTS

|           |         |          |
|-----------|---------|----------|
| 1,382,682 | 11/1964 | France.  |
| 643,834   | 6/1964  | Belgium. |

JOSEPH L. SCHOFER, *Primary Examiner.*

HARRY WONG, *Assistant Examiner.*